

May 25, 1965

K. K. HUMPHREYS

3,184,952

METHOD AND APPARATUS FOR DETERMINING COKE STRENGTH

Filed July 14, 1961



INVENTOR

KENNETH K. HUMPHREYS

By *Donald G. Dalton*  
Attorney

1

3,184,952

**METHOD AND APPARATUS FOR DETERMINING  
COKE STRENGTH**Kenneth K. Humphreys, Wilkinsburg, Pa., assignor to  
United States Steel Corporation, a corporation of New  
JerseyFiled July 14, 1961, Ser. No. 124,072  
4 Claims. (Cl. 73—12)

The present invention relates to a novel method and apparatus for testing particulate matter at normal or elevated temperatures. More particularly, it relates to a method and apparatus for determining the strength of solid metallurgical fuels under conditions similar to those occurring in a blast furnace.

In the blast-furnace process material charged to the furnace is called the burden and includes principally iron ore, flux, coke and scrap. Metallurgical coke and other fuels, such as charcoal and coal, are commonly used as (1) sources of heat and reducing gas, (2) for maintaining burden permeability and (3) for supporting the weight of the other burden materials during their descent through the furnace shaft. These fuels, therefore, must be capable of maintaining their integrity until they are consumed by combustion and other chemical reactions or by solution in the metal pool at the base of the furnace.

As the solid fuel particles reach the tuyere zone of a blast furnace, they are subjected at high temperatures to extremely turbulent motion imparted by the hot blast air entering from the tuyeres to create so-called blast furnace raceways. If the particles are not of sufficient strength at these temperatures to withstand this motion, they will become degraded and thus no longer effective for providing the required support for the furnace burden. Hence, the burden movement becomes erratic by sticking or hanging, thereby upsetting furnace operation. This also results in small fuel particles collecting in the void spaces within the burden above the raceways to reduce its permeability, thereby increasing the pressure drop through the burden and decreasing the amount of air which can be blown through the burden. This renders the furnace difficult to control and thus causes inefficient operation and decreased production. Hence, it is important that only solid fuels having sufficient physical strength at elevated temperatures be charged to a blast furnace.

It is, therefore, an object of my invention to provide a method and apparatus for determining the physical strength of solid metallurgical fuels under conditions similar to those existing in a blast furnace.

A more specific object of my invention is to provide means for heating a sample of solid fuel to a temperature equal to that existing in the tuyere zone of a blast furnace and then subjecting the heated material to degrading action similar to that occurring within this zone.

Methods have been proposed for testing and predicting the strength of coke and other solid fuels to avoid charging fuel of inferior strength to the blast furnace. These tests generally consist of abrading, e.g., ASTM Tumbler Test for Coke, Designation D294-50; impacting, e.g., ASTM Drop Shatter Test for Coke, Designation D141-48; or otherwise subjecting coke samples to degrading forces. A relative-strength index is then reported, usually as the weight percent of original coke passing or being caught on a sieve of some arbitrary size.

These tests have the following common limitations:

(1) They are not conducted at temperatures representative of those experienced in the lower portion of a blast-furnace stack where mechanical stresses are greatest and where temperature effects are most pronounced. At these temperatures, coke is supporting its maximum weight load and in addition is subjected to violent motion

2

and severe impact and abrasive forces caused by turbulence in the coke bed because of the high-velocity air jets issuing from the tuyeres.

(2) The rate of momentum transfer between coke particles in existing tests is not comparable to that in a blast-furnace tuyere zone. The air jets in this area, having velocities greater than 200 feet/second, impart a much larger kinetic energy to the particles than that imparted to them by existing tests.

10 (3) Because they are conducted at ambient temperatures rather than at blast-furnace operating temperatures, coke-strength indices obtained from existing low-temperature tests do not necessarily predict coke strength in the blast furnace. Coke is a heterogenous mixture of many materials and does not necessarily retain its low-temperature strength characteristics at elevated temperatures. Cokes possessing equal strengths at ambient temperatures often vary widely in strength at elevated temperatures.

(4) Because they do not exert a degrading force on coke 20 at the same temperatures and by a similar mechanism as that occurring in the blast furnace, existing test indices frequently do not correlate with blast-furnace performance. Coke having high strength according to some existing tests, frequently degrades excessively in the blast furnace.

(5) In addition, existing tests are time-consuming and 25 difficult to perform. Large samples must be tested and a number of duplicate tests must be performed to obtain consistent strength indicates for a given coke or other solid fuel.

The deficiencies enumerated above are substantially 30 eliminated by the use of my invention. A complete understanding of the invention may be obtained from the following detailed description and explanation which 35 refer to the accompanying drawing illustrating the present preferred practice. The single figure of the drawing is a diagrammatic representation of apparatus for carrying out the method of my invention. The apparatus as there shown may be considered as two interconnected 40 conduits or pipes. In the one conduit, the sample of screened particles is heated to simulate an operating temperature. The heated sample is then transferred to the other conduit and entrained in a horizontally-moving high-velocity gas stream. The entrained sample is then 45 impinged tangentially against an inner wall of a circular obstruction and is thereby abraded in a rotary motion to simulate an operating condition. Preferably, the entrained sample travels in a horizontal conduit between the areas of entrainment and impingement.

50 Referring now in detail to the drawing, a sample of the screened particles 10 to be tested, is admitted to conduit or pipe 12 through a capped opening 14. The particles are then pushed to the position shown, in a tube-type furnace 16 by a pusher having a heat-resisting head 55 18 that preferably fits snugly in conduit 12. The head, acting as a piston, is carried on a reciprocable, heat-resisting rod 20, preferably of stainless steel. The rod passes through a packing gland 22 in conduit 12. Furnace 16 which may be gas-fired or electrically heated, here 60 comprises a refractory tube 24 partially surrounded by insulation 26, the portion thereof in open chamber 28 being heated by a series of electrical heating elements 30. Spring-loaded flanges 32 permit expansion and contraction of tube 24, as an integral part of conduit 12, the 65 remainder thereof being heat resistant pipe, preferably of stainless steel.

During heating of sample 10, nitrogen or any other 70 suitable inert gas may be introduced to conduit 12 through a pipe 34 to prevent combustion of sample 10. When the sample has been heated to the preferred temperature, rod 20 is advanced, the sample being pushed along conduit 12 and dropped on a reciprocable, quick-opening

valve 36, which is thereafter opened to transfer the sample from conduit 12 to conduit 38. Conduit 12 may be straight, permitting rod 20 to push the sample into conduit 38 and directly into the gas stream.

A rapidly-moving stream of air or inert gas, supplied by blower 40, is passed through conduit 38 to entrain the particles of sample 10 and to impart to them kinetic energy substantially equal in magnitude to that which they would receive in the tuyere zone of a blast furnace. The outlet of blower 40 is connected to a conduit 42, having therein a device to measure gas-flow rate, for example, an orifice plate 44 with taps on either side thereof connected to a differential pressure gage 46. A by-pass gate valve 48, with a manually or automatically controlled opening permits adjusting the gas flow in conduit 42 and thereafter in conduit 38 to which it is connected.

Conduit 38 is connected tangentially to and near the open top of an abrasion and impact cylinder 50, supported on a stand 52. Cylinder 50 serves as an obstruction or abrasion means which will permit the particles of sample 10 to strike or impinge against the inner wall and rotate about the perimeter of cylinder 50 and to proceed therearound in a rotary-motion abrasion to simulate the abrasive action which my studies have indicated as being comparable to that taking place in the raceways at the tuyere zone of a blast furnace. The motion of the sample becomes slower as the energy of motion dissipates and the sample particles settle to the bottom of the cylinder. The separated gas flows upward from the open top of the cylinder, which may be covered by a screen 54 to prevent loss of fine sample particles with the gas. A conical or funnel-shaped bottom or container 56, integral with cylinder 50 serves to receive sample 10. The conical shape of container 56 presents a resistance to downward flow of the gas and thereby induces it to seek the upward path of least resistance. The bottom valve or closure 58 of the container 56 is fitted with a pipe 60 for the introduction of nitrogen or other suitable inert gas to prevent or minimize combustion of the sample. The cooled sample is collected for rescreening and weighing. If desired, the sample may be returned to the apparatus for further testing.

A specific example of the practice of the invention, giving quantities involved, is set forth below.

The example has as an object the determination of the suitability of coke for use in an experimental blast furnace by simulating known operating conditions: (1) a tuyere-zone temperature of about 3200° F., and (2) an air-blast linear velocity of about 440 feet per second in the nose of the tuyeres. The latter creates a high-speed rotary motion of entrained solid particles, approximately in a circular cross-section having about an 18" diameter, wherein the particles abrade against each other and against less-agitated solid burden particles.

A five pound sample of blast-furnace coke, screened to a size such that its particles are retained on 1" and pass through 1½" screens, was charged through opening 14 to conduit 12 and pushed into refractory tube 24 in furnace 16. It was heated to about 3200° F. in an atmosphere of nitrogen, supplied through pipe 34. When the heating was substantially completed, blower 40 was started, and valve 48 adjusted to provide an air flow of about 440 feet per second in the 3" conduit 38. Pusher rod 20 was thereafter advanced and the heated sample pushed through conduit 12 until it fell on valve 36. Opening of this valve dropped the sample into conduit 38 where it became entrained in the air stream, being thereafter impinged tangentially against the circular wall of an 18" diameter cylinder 50, to induce a rotary-motion abrasion of the entrained sample. As their kinetic energy was dissipated thus separating them from the air, the coke particles dropped and the separated air left the open top of cylinder 50 through screen 54. Having been entrained in the air stream for about 0.1 second, the sample thereafter gathered in the conical bottom 56 to

cool in nitrogen, pumped in through pipe 60. The sample was thereafter collected, rescreened and weighed. A relative measure of the physical strength of the sample may then be determined and reported as the ratio of the weight of particles retained on a 1" screen after the test to the original weight retained on a 1" screen. This ratio is a good index for comparing the relative suitability of various fuels for use in the blast furnace. That fuel having the highest ratio being the stronger and therefore the better fuel. For example, for 5# samples, after-test weights of 4.5# and a ratio of

$$\frac{4.5}{5.0} = 0.9$$

indicates an extremely strong coke; 3.8#, 0.76 ratio, a moderately strong coke; 2.1#, 0.42 ratio, an extremely weak coke.

I have found that when testing samples according to my invention, the results are reproducible within limits of  $\pm 3\%$ . Error caused by combustion of the particles is negligible in the short time interval that the samples are in contact with the air blast. Maximum retention time of the particles in the air stream is 0.1 second or even less when simulating the highest jet velocities encountered in blast-furnace operation. Cooling of the particles while they are in the blast line is also negligible.

While the above example illustrates a preferred method of operation, other conditions of operation may be used without departing from the spirit of the invention. The sample may be heated to any temperature existing in the blast-furnace stack to determine the strength of a sample in this area. The heating step may be eliminated to determine the breakage characteristics of the fuel during handling. The impact-abrasion cylinder 50 may be replaced by a conical or funnel-shaped means or by a box or flat plate when determining the resistance of the sample to impact forces at ambient or elevated temperatures. The air stream in the air-blast pipe may be heated in addition to heating the sample, to minimize heat losses therefrom. The invention may also be used to test solid materials other than metallurgical fuels.

It will be apparent that apparatus changes may then be made to effect the desired result. The conduits 12 and 38 need only be large enough to conveniently accommodate the sample particles. The blower should have a capacity to deliver the velocity and volume of gas or air required. The diameter of an impact-abrasion cylinder may be larger or smaller, as required by operating conditions. In actual operation of blast furnaces, it has been determined that the race way diameters at tuyere level will vary between about 12" and 48". The variations depend on factors including blast furnace geometry, air flow rate and size of materials. The impact-abrasion cylinder diameter and fuel-test conditions should then be within the range of operating conditions. This should also be the case when testing materials other than blast furnace coke.

Many of the deficiencies in prior-art coke testing, as being non-indicative of blast furnace operating conditions, are substantially eliminated by the use of my invention. In accordance therewith, testing is performed at the temperatures existing in the tuyere zone of the blast furnace. In addition, strength indices may be obtained at any lower temperature level if desired, as a measure of coke strength in the upper regions of the blast-furnace stack. Similarly testing may be performed at ambient temperatures to obtain an estimate of fuel breakdown during handling prior to charging. Testing is performed at jet and particle velocities equivalent to those occurring in a blast-furnace tuyere zone; thus the rate of momentum transfer and abrasion occurring between particles in a blast furnace is simulated. In this way I can determine which fuels should perform well in a blast furnace and which may adversely affect furnace operation. My invention does not require that large coke samples be tested to obtain

consistent results. A single strength determination of a few pounds of coke is usually sufficient. Testing time and the quantities tested are, therefore, minimized. My invention also has the advantage of being capable of adjustment to any desired set of blast-furnace operating conditions. This flexibility permits accurate determination of coke strength at such conditions, and also permits the use of my invention for a wide variety of other strength-testing purposes on a wide range of solid materials.

Although I have disclosed herein the preferred practice and apparatus of my invention, I intend to cover as well as any change or modification therein which may be made without departing from the spirit and scope of the invention.

I claim:

1. A method of testing a charge of particles having a predetermined minimum starting size substantially greater than the size of particles when disintegrated to a powder, to determine their resistance to being abraded to smaller particles, comprising placing a charge of particles of at least said minimum starting size in a horizontally disposed cylinder, applying heat to the cylinder, then, after the charge has been heated to a predetermined temperature, pushing a piston through said cylinder and quickly displacing the charge therefrom with minor abrasion thereto, immediately injecting the charge into an impact chamber in a stream of compressed gas and controlling the force exerted by said gas to abrade the charge therein to a limited degree, but insufficient to effect impact-disintegration thereof to a powder, and finally collecting the abraded charge.

2. A method as defined in claim 1 characterized by the charge being blast furnace coke, all the particles thereof having at least a minimum size usable in a blast furnace, heating said charge to about 3200° F. in an inert atmosphere and entraining said heated particles in an air stream moving at about 440 feet per second.

- 5 3. Apparatus for testing a charge of particles having a predetermined minimum starting size substantially greater than the size of particles when disintegrated to a powder, to determine their resistance to being abraded to smaller particles, comprising a cylinder disposed substantially horizontally, a piston reciprocable therein, a heating chamber through which the cylinder extends, an impact chamber having an injector gas-supply pipe connected thereto, a pipe connecting one end of said cylinder to said injector pipe and means connected to said injector pipe adapted to supply thereto a stream of compressed gas having a controlled force to abrade the charge in said impact chamber to a limited degree, but insufficient to effect impact-disintegration thereof to a powder.
- 10 15 4. Apparatus as defined in claim 3 characterized by said impact chamber comprising a vertical, open-top, funnel-shaped receptacle, having a screen over said top and a valve at the bottom thereof.

#### References Cited by the Examiner

##### UNITED STATES PATENTS

|              |       |                 |       |          |
|--------------|-------|-----------------|-------|----------|
| 2,242,796    | 5/41  | Stockton        | ----- | 241—17   |
| 2,515,542    | 7/50  | Yellott         | ----- | 241—5 X  |
| 2,768,938    | 10/56 | Martin          | ----- | 241—5 X  |
| 2,853,241    | 9/58  | Gindoff et al.  | ----- | 241—40 X |
| 2,864,560    | 12/58 | Carkeek et al.  | ----- | 241—17 X |
| 2,905,321    | 9/59  | Hitchner        | ----- | 73—12 X  |
| 2,983,453    | 5/61  | Bourguet et al. | ----- | 241—5 X  |
| 30 2,995,026 | 8/61  | Schmidt         | ----- | 73—12    |

##### FOREIGN PATENTS

1,094,977 12/54 France.

35 RICHARD C. QUEISSE, Primary Examiner.  
ROBERT L. EVANS, Examiner.